

Oct. 25, 1932.

C. L. MCKESSON  
EMULSIFIED ASPHALT PENETRATION PAVEMENT  
AND PROCESS OF CONSTRUCTING THE SAME  
Filed Dec. 29, 1928

1,884,795



Fig. 1.



Fig. 2.



Fig. 3.

*Claude L. McKesson* Inventor

## UNITED STATES PATENT OFFICE

CLAUDE L. MCKESSON, OF OAKLAND, CALIFORNIA, ASSIGNOR TO AMERICAN BITUMULS COMPANY, OF SAN FRANCISCO, CALIFORNIA, A CORPORATION OF DELAWARE

EMULSIFIED ASPHALT PENETRATION PAVEMENT AND PROCESS OF CONSTRUCTING  
THE SAME

Application filed December 29, 1928. Serial No. 329,302.

My invention relates to the construction of a bituminous pavement somewhat resembling hot asphaltic penetration macadam but which is free from defects inherent to that type and which embodies all of the superior qualities usually found only on hot plant mixed asphalt concrete pavement.

More specifically the objects which I accomplish are the elimination of large voids particularly in the lower portion of the pavement and excesses of bituminous binder which necessarily results from the use of coarse rock and hot asphalt in the first course of the penetration type as heretofore constructed. These unavoidable defects frequently lead to the failure of the pavement. By my method of construction I secure a dense pavement of interlocking stone particles each of which is uniformly coated with a thin efficient thickness of pure asphalt binder. The under side of my pavement is thoroughly and efficiently sealed against the entrance of moisture or mud from subgrade and the surface of the pavement is likewise sealed to prevent the entrance of moisture falling on the surface.

The foregoing and other beneficial results are attained in the following manner:

My invention will be clearly understood by reference to the following description and to the accompanying drawing in which Fig. 1 represents a section of pavement during the first stage of construction, in which (1) indicates the subgrade which may be of earthy material, brought to grade and compacted, (2) shows a layer of stone dust or fine sand, and (3) a layer of crushed rock or gravel graded from maximum to minimum preferably with exclusion of fines.

Fig. 2 shows the second stage of construction in which the numerals (1), (2) and (3) are the same as above except that the layer of crushed rock (3) is shown coated with bituminous emulsion. The numeral (4) indicates a layer of bituminous emulsion collected and lying on the layer of stone dust (2). The numeral (5) indicates a top coating of screenings placed on the graded aggregate (3) after the application of the bituminous emulsion.

Fig. 3 shows the completed pavement, the

corresponding numerals being the same as in Fig. 2. In this figure is illustrated the final seal coat (6) which consists of an application of Portland cement or stone dust swept into the interstices of the compacted screenings (5) and covered with bituminous emulsion.

The first stage in the production of this new and novel type of pavement is the placing on the subgrade (1) of a thin layer (2) of stone dust and stone chips or of sand, preferably fine. On this is spread a layer of crushed rock or gravel (3) having an uncompacted thickness of one fifth to one third more than the desired finished thickness of the pavement to be built. This crushed rock or gravel is graded in size from a maximum to a minimum. The maximum size is not arbitrarily fixed except that the largest dimension of the coarse particles should not exceed three fourths of the finished thickness of the pavement. The minimum size of particles is very important. Particles which pass a U. S. standard 10 mesh sieve are excluded where best results are to be secured. In usual practice material is not used which will not pass a screen having circular openings of a diameter of half of the finished thickness of the pavement. The grading between the maximum limit selected and the minimum size limit as above set forth which is most satisfactory is one which will reduce the voids to a minimum. Usually the voids can be brought to about thirty per cent in the loose uncompacted material. Satisfactory results may be had with a grading which follows either the original or the modified Fullers maximum density formula or by means of so-called jump gradings in which certain sizes are omitted.

After the material is spread on the subgrade it is turned with blades and disc or spring tooth cultivators until thoroughly and uniformly mixed and blended. Segregated spots of fine or coarse material must be entirely corrected at this stage of the construction. During the blading and cultivating operations, stone dust or dirt which may have remained in the material falls to the bottom.

The surface of the material is then shaped with a blade to conform with the finished

55

60

65

70

75

80

85

90

95

100

contour of the road. After the graded crushed rock or gravel is thus prepared, bituminous binder in the form of an aqueous asphaltic emulsion is applied in sufficient quantity to entirely penetrate and permeate the layer of graded crushed rock or gravel (3) and with some excess (4) which collects beneath this material on the layer of stone dust and chips or sand first placed.

10 The character of this emulsion is essential to the successful construction of my pavement. A suitable emulsion must have a very low viscosity, preferably less than a specific viscosity of two (Engler). Such emulsions 15 are now made commercially using asphalt and water with small additions of caustic soda, oleic acid or other emulsifying agents, but to my knowledge emulsions were not used in the construction of the type herein 20 described prior to my invention. A desirable emulsion should contain fifty per cent or more of asphalt, the remainder being water and emulsifying agent.

25 The emulsion is preferably applied with pressure distributors in two or more applications. The amount required is usually about one-half gallon per square yard per inch of finished thickness, assuming the emulsion to have an asphalt content about as stated above.

30 After the emulsion has been applied the surface of the pavement is lightly covered with screenings (5) and is then rolled with a suitable roller until it is fully compressed 35 and until it is firm and unyielding. During the first rolling soon after the emulsion has been spread, the pavement is plastic under the roller and is readily shaped to the desired contour. Usually the final rolling can 40 not be done until one or more days after the emulsion has been spread, the lapse of time being necessary to allow the emulsion to "break" or "set".

45 After the pavement thus constructed has been fully and finally compacted it is given a seal coat (6). This consists of an application of Portland cement or stone dust swept into the interstices in the surface of the pavement and then covered with a light 50 application of emulsified asphalt. Portland cement is preferable for the seal coat because it quickly draws moisture necessary for hydration from the emulsion thereby breaking the emulsion. The Portland cement hardens 55 in the interstices into which it has been swept, renders the pavement waterproof and at the same time prevents subsequent displacement of rock particles in the surface of the pavement. Stone dust if used also takes 60 moisture from the emulsion and in time absorbs the surplus asphalt in the seal coat. The amount of Portland cement or stone dust used is the amount which can be swept into surface interstices in the pavement and varies 65 under different conditions.

It will be noted that this pavement differs from usual penetration macadams in that it does not use different sizes of stone in successive layers beginning with large stone openly graded, followed by key rock, etc. 70 It also has a distinct advantage and effects great economy in that hand labor is almost entirely eliminated. It has the additional advantage of greater smoothness because of its plasticity when first rolled. High spots, 75 bumps and low spots are corrected by rolling at this stage. With types heretofore used, it is well known that irregularities of this kind cannot usually be eliminated by rolling but must be avoided by careful correction 80 after the first rolling and before hot asphalt has been applied.

85 The thickness of a pavement constructed according to my method is limited only by the ability of the roller to properly compress the rock. In a test I have readily penetrated one foot of material graded from  $\frac{3}{8}$ " mesh to 10 mesh with emulsion and have fully coated the particles with asphalt. Such material is finer, as to maximum size, than 90 would generally be used.

95 The pavement herein described offers an added economy in that it utilizes the entire product of the crusher ranging from the maximum size to stone dust.

100 The mat formed on the bottom of the pavement consisting of stone dust and asphalt effectively prevents mud and water from entering the pavement from the under side, a common cause for failure in ordinary penetration macadams in which the coarse base stone is usually poorly filled with screenings due to the inability to get screenings through the carpet of hot asphalt which collects in the upper interstices base stone. 105

Having thus described my invention what I claim as new and desire to secure by Letters Patent is:

110 1. A pavement consisting of stone particles graded from maximum to a minimum size which excludes material passing a ten mesh sieve screen, a coating of emulsified asphalt on the stone particles and a seal coat of stone dust and asphalt emulsion on the under side of said pavement.

115 2. A pavement consisting of a layer of emulsified asphalt covered stone dust and screenings adjacent to the subgrade, a layer of compressed stone above said layer of stone dust, forming the main body of said pavement, said compressed stone being graded in size from a maximum and substantially free from fines to a minimum, and a coating of emulsified asphalt on said stone particles.

120 3. The process of constructing a pavement comprising placing a layer of stone dust and screenings upon a subgrade, upon this placing a layer of crushed rock graded from a maximum to a minimum size, composing the 125 main body of the pavement, penetrating the 130

- said crushed rock with an aqueous emulsion of asphalt, a portion of which is allowed to pass through the crushed rock and collect on the stone dust beneath forming thereby an under seal, and finally rolling the crushed rock until it is firm and unyielding. 5
4. The process of constructing a pavement comprising placing a layer of stone dust and screenings upon a subgrade, upon this placing a layer of crushed rock graded from a maximum to a minimum size, composing the main body of the pavement, penetrating the said crushed rock with an aqueous emulsion of asphalt, a portion of which is allowed to pass through the crushed rock and collect on the stone dust beneath forming thereby an under seal, rolling the crushed rock until it is firm and unyielding, applying a seal coat consisting of Portland cement sufficient in quantity to fill interstices in the surface of the pavement and finally coating the surface with emulsified asphalt. 10
5. The process of constructing a pavement comprising placing a layer of road material graded from a maximum size to a minimum size which excludes all material passing a ten mesh screen, of penetrating the said material with an aqueous emulsion, a portion of which is allowed to pass through the material and collect beneath forming thereby an under seal, rolling the material until it is firm and unyielding, finally applying a seal coat consisting of Portland cement sufficient in quantity to fill interstices in the surface of the pavement and by coating the surface with emulsified asphalt. 15
6. The process of constructing a pavement comprising placing a layer of fine road material on a subgrade, placing thereon a layer of mineral aggregate substantially free from fine material, applying to the surface thereof an aqueous emulsion of bituminous binder in quantity sufficient to coat the aggregate and collect on the fine material beneath, thereby forming an under seal, and finally compacting the coated aggregate. 20
7. The process of constructing a pavement comprising placing a layer of fine road material on a subgrade, placing thereon a layer of mineral aggregate substantially free from fine material, applying to the surface thereof an aqueous emulsion of bituminous binder in quantity sufficient to coat the aggregate and collect on the fine material beneath, thereby forming an under seal, compacting the coated aggregate until firm and unyielding, and finally applying a top seal of fine road material and emulsified bitumen. 25
8. The process of constructing a pavement which comprises placing a layer of mineral aggregate substantially free from material passing a ten mesh screen, applying to the surface thereof an aqueous emulsion of bituminous binder in quantity sufficient to coat the aggregate and collect beneath, thereby 30 forming an under seal, compacting the aggregate until firm and unyielding, applying a seal coat of fine road material in quantity sufficient to fill interstices in the surface, and finally coating the surface with emulsified bitumen. 70
9. A pavement comprising mineral aggregate substantially free from fine material, a coating of emulsified bitumen on said mineral aggregate and a seal coat of emulsified bitumen and fine material on the under side of said pavement. 75
10. A pavement comprising graded mineral aggregate substantially free from fine material, a coating of emulsified bitumen on said mineral aggregate, a seal coat of emulsified bitumen on the underside of said pavement and a seal coat of fine road material and emulsified bitumen on the surface. 80

CLAUDE L. MCKESSON. 85

90

95

100

105

110

115

120

125

130

CERTIFICATE OF CORRECTION.

Patent No. 1,884,795.

October 25, 1932.

CLAUDE L. McKESSON.

It is hereby certified that error appears in the printed specification of the above numbered patent requiring correction as follows: Page 2, line 123, claim 2, strike out the words "to a minimum" and insert the same after the word "maximum", in line 122; page 3, line 32, claim 5, strike out the word "finally", and line 35, for "by" read "finally"; and that the said Letters Patent should be read with these corrections therein that the same may conform to the record of the case in the Patent Office.

Signed and sealed this 24th day of January A. D. 1933.

M. J. Moore,  
Acting Commissioner of Patents.

(Seal)